

# UNITED STATES PATENT OFFICE.

FREDERICK GRAFFE, JR., OF FORT WAYNE, INDIANA.

## COMPOUND FOR CLEANING JEWELRY.

SPECIFICATION forming part of Letters Patent No. 425,668, dated April 15, 1890.

Application filed April 4, 1889. Serial No. 306,000. (Specimens.)

*To all whom it may concern:*

Be it known that I, FREDERICK GRAFFE, Jr., a citizen of the United States, residing at Fort Wayne, in the county of Allen and State 5 of Indiana, have invented certain new and useful Improvements in Cleansing Preparations for Jewelry, &c.; and I do hereby declare the following to be a full, clear, and exact description of the invention, such as will 10 enable others skilled in the art to which it appertains to make and use the same.

The cleaning of jewelry with the preparations heretofore used for that purpose and in the manner heretofore practiced has been a 15 matter requiring considerable time and labor. With the view of simplifying the operation and at the same time obtaining better results I have invented and prepared a new mixture, which is easily applied and used, and when 20 used in the manner hereinafter described will effectually clean all kinds of jewelry in the shortest time and with the least expenditure of labor, and will restore to the same its original brightness and luster.

25 The mixture is a solution composed of the following ingredients and in the proportions set forth, viz:

|                      | Parts. |
|----------------------|--------|
| Potassium bitartrate | 20     |
| Rouge                | 2      |
| Liquor potassæ       | 50     |
| Water                | 25     |
| Perfume              | 3      |
| 35 Total             | 100    |

40 The perfuming ingredient adds nothing to the cleansing properties of the mixture and is used merely to give a pleasant odor when using the preparation. Any preferred per-

fuming substance or preparation may therefore be used. That which I prefer is itself a mixture made up of the following ingredients, viz: oil of lemon, two and one-half drams; oil of lavender-flower, fifteen drams; 45 oil of pimento, fifteen drams; alcohol, one pint.

The manner of applying and using this preparation is as follows: Take an ordinary tooth-brush, the softer the better, and wet thoroughly by dipping in water; then pour on 50 a small quantity—say eight or ten drops—of the cleaning preparation and draw over a cake of soap; rub the article thoroughly with the brush so moistened and prepared, and then rinse well in clear water; then place in 55 fine sawdust, the finer the better, and stir around in the same or shake well, and leave it a few minutes to dry. When dry, the dust will fall off and the article will be as clean and bright as when new.

6c In cleaning delicate articles—such as small settings which will not bear rubbing with the brush—it will be sufficient to press the brush gently upon the same, repeating the operation until the settings are thoroughly 65 moistened; then rinse and dry as above.

Having now described my invention and the manner of applying and using the same, I claim—

70 The hereinbefore-described cleansing mixture for cleaning jewelry and similar articles, composed of potassium bitartrate, rouge, liquor potassæ, and water, in about the proportions set forth.

75 In testimony whereof I affix my signature in presence of two witnesses.

FREDERICK GRAFFE, JR.

Witnesses:

J. W. SMITH, Jr.,

C. W. ORR.